

## UNITED STATES PATENT OFFICE

2,264,490

## PROCESS FOR TREATING TEXTILES

Ernst Waltmann, Krefeld, Germany, assignor to  
Heberlein Patent Corporation, New York, N. Y.,  
a corporation of New York.

No Drawing. Application December 31, 1937, Se-  
rial No. 182,915. In Germany January 2,  
1937

4 Claims. (Cl. 8—113)

This invention relates to treating textile materials and particularly to dyeing them and rendering them water-repellent and to products obtained thereby. It also relates to chemicals and processes for producing the same, useful in so treating the textile material.

I have found in accordance with my invention that for the purpose of preparing fibers for dyeing, I may treat them with ethers containing a basic nitrogen atom. Such treatment in the case of cotton or other cellulosic material is capable of animalizing the material, that is of imparting to it characteristics of animal fibers such as wool, whereby the material so treated can be dyed with acid dyes. In addition I have found in accordance with my invention that where the compounds employed for treatment are of higher molecular weight there is imparted to the fibers, in addition to the animalizing, a permanent power of resistance to wetting by water.

Processes have been already proposed for introducing into viscose solution an addition of casein, albumen or other nitrogenous substances, and it has also been proposed to treat alkali or alkaline earth compounds of cellulose with alkalizing nitrogenous agents. These proposed processes, however, are either expensive or do not produce a uniform result in the fibers treated and are not practical for large scale production.

An important object of my invention accordingly is to provide an improved process of the kind described which shall do away with at least some of the difficulties found in the heretofore proposed processes and to produce a series of improved products.

The invention comprises the novel products as well as the novel processes and steps of processes according to which such products are manufactured, the specific embodiments of which are described hereinafter by way of example and in accordance with which I now prefer to practice the invention.

In carrying out my improved process I employ others as stated above. These compounds must contain in addition to the active group which effects the action with the cellulose, an aliphatic or cyclic radical of at least four carbon atoms and besides in this radical at least one basic nitrogen atom.

The ethers can be brought into water-soluble condition in the form of their quaternary ammonium compounds so that the entire treatment is carried out in an aqueous solution. If the ethers contain aliphatic, aliphatic-aromatic or alicyclic radicals containing at least ten carbon atoms in a straight chain, there is imparted to the fibers in addition to the animalization also a permanent power of resistance to wetting with water.

Fibers of cellulosic material which have been treated by such agents in accordance with my invention are well suited to mixture with wool fibers. The mixed fabrics manufactured therefrom can be dyed in the usual manner with dyes which incline to acidity, whereby a considerable saving in dye is attained, as well as saving in the dyeing process.

Falling under the class of ethers used for impregnating the textile material and which cause it to become water-repellent upon baking are quaternary ammonium salts of methyl halogen ethers containing a basic nitrogen atom other than that of said ammonium radical, and also containing an aliphatic radical of at least 10 carbon atoms, said basic nitrogen atom being attached to said aliphatic radical.

Although the process so far as it concerns dyeing is particularly directed to rendering cellulosic material capable of being dyed by acid dyes, nevertheless wool itself may be treated by any of the compounds herein mentioned and if the compounds of my invention contain more than ten carbon atoms in a straight chain they will produce in the wool in addition a water-repellence.

The following are examples of embodiments of the manner in which I now prefer to practice the invention in the treatment of textiles. It is to be understood that the invention is not limited thereto except as indicated in the appended claims.

## Examples

1. Spun viscose rayon (cell wool flock) is impregnated at room temperature by an aqueous solution which contains per liter 15 grams of the quaternary pyridinium salt of the methyl chloride derivative which has been obtained as described below by double decomposition of octadecane nitile  $C_{17}H_{35}CN$  with trioxymethylene and hydrochloric acid gas. After the impregnation the material is centrifuged, dried at  $70^{\circ} C.$  and exposed for about 6 hours to a temperature of about  $90^{\circ} C.$  ( $194^{\circ} F.$ ). The viscose spun rayon which has been treated in this way is dyed by treating it with:

|                                                             | Grams per liter |
|-------------------------------------------------------------|-----------------|
| Polar Red 3 B Schulz Dyestuff table 7, edi-<br>tion No. 475 | 0.1             |
| Sodium sulphate ( $Na_2SO_4$ )                              | 5               |
| Acetic acid                                                 | 1               |

at a temperature of  $90$ — $100^{\circ} C.$ , and the dyed material at the same time manifests water-repelling properties.

2. Viscose spun rayon (cell wool flock) is impregnated at room temperature in an aqueous solution which contains per liter 20 grams of the quaternary pyridine salt of the methyl chloride compound prepared from octadecane cyano-

hydrin  $\text{CH}_3(\text{CH}_2)_{15}\text{CH}(\text{OH})\text{CN}$  trioxymethylene and hydrochloric acid gas in accordance with the directions of French Patent No. 743,594. The bath also contains besides per liter 5 grams of sodium acetate. After impregnation the material is centrifuged, dried and exposed for about 6 hours to a temperature of about 90° C. (194° F.). The spun rayon material which is treated in this way is dyed in the same way mentioned in Example 1. The dyed material at the same time 10 manifests water-repelling properties. The dye is more light fast than is obtained where the sodium acetate is omitted.

3. 20 parts of the quaternary ammonium compound which is prepared by double decomposition of trimethylamine and methyl chloride ether of the formula:



are stirred to a paste with 40 parts of hot water of about 50° C. and are added to 1000 parts of a viscose solution having 5% of cellulose. The whole is homogeneously mixed and is spun in well-known fashion. The coagulation bath consists in the main of sulphuric acid (8-10%) with the addition of ammonium sulphate and/or other salts and glucose at a temperature of 40° C. Thereafter the thread is heated at 30° C. for 60 minutes and thereupon shows water repelling properties. It may be dyed in the same manner as set forth in Example 1 and the dyed fiber thereafter exhibits water repelling properties.

The result of the treatment of the textiles in the manner above described is to cause an action to occur between the textile and the treating substance, etc., which produces water-repellence in the textile. The dye baths employed in the preceding examples are also suitable for the usual wool dyeing, and the shades obtained are similar.

The dyeing step may be omitted in Examples 1 to 3 inclusive. If omitted the undyed material still exhibits the desired water-repelling properties.

The following are examples for methods of preparing the chemicals described herein:

4. Dry hydrochloric acid gas is introduced at ordinary temperature into a mixture of 266 grams of octadecan-nitrile  $\text{C}_{17}\text{H}_{35}\text{CN}$ , 500 grams of benzol and 60 grams of trioxymethylene until the formation of the chloromethyliminoether has taken place. The benzol and the surplus hydrochloric acid are removed by suction in a vacuum at a temperature of about 40 to 50° C. and the chloromethyl compound is stirred with 100 grams of dry pyridine. The water-soluble quaternary pyridinium salt of chloromethyliminoether is produced. The reaction is believed to proceed as follows:



5. Octadecylene  $\text{CH}_3(\text{CH}_2)_{15}\text{CH}:\text{CH}_2$  is stirred 70 with a diluted solution of subchloric acid  $\text{HOCl}$  in water until octadecylchlorhydrine is formed



The obtained octadecylchlorhydrine is dried and then heated in an autoclave with an excess of diethylamine  $(\text{C}_2\text{H}_5)_2\text{NH}$  4 hours to 150° C. The hydrochloric acid salt of octadecyl aminoalcohol is formed according to the equation:



The last compound is combined in a known manner with trioxymethylene and hydrochloric acid gas whereby the chloromethyl ether of octadecylaminoalcohol is formed. By treating this compound with a tertiary amine, such as, trimethylamine  $(\text{CH}_3)_3\text{N}$ , the corresponding quaternary ammonium compound is formed having the formula:



The process of the invention, particularly as set forth in the specific embodiments, may be carried out with simple apparatus at relatively small expense and in a relatively short time. The textile products show an improved appearance, their feel as compared with similar untreated material is not substantially altered, and they have a high degree of water-repellence which does not rapidly disappear upon cleansing by laundering or otherwise of the materials produced.

Subject matter described but not claimed herein is claimed in my copending application Serial No. 267,317, filed April 11, 1939.

The term "textile material" as herein employed is intended to include wool and silk as well as cellulose-containing material. The expression "cellulosic-material" as herein employed is intended to cover fibers, yarns, fabrics or other forms of cotton, jute, linen, hemp or rayon including viscose, cuprammonium, or other precipitated cellulose or derivatives of cellulose such as acetyl cellulose, so long as such materials still contain a hydroxyl group or groups that will act with the etherifying and other agents herein employed to produce the dyeing effects and/or water repellent effects herein described.

While the invention has been described in detail according to the preferred manner of carrying out the process, it will be obvious to those skilled in the art after understanding the invention, that changes and modifications may be made therein without departing from the spirit or scope of the invention, and it is intended in the appended claims to cover all such changes and modifications.

What is claimed as new and desired to be secured by Letters Patent is:

1. A process for rendering textile material water-repellent and to improve its affinity for acid dyes which comprises impregnating textile material with a quaternary ammonium salt of a methyl halogen ether containing a basic nitrogen atom other than that of said ammonium radical, and also containing an aliphatic radical of at least 10 carbon atoms, said basic nitrogen atom being attached to said aliphatic radical, and baking the impregnated textile material at a temperature sufficient to cause the material to become water-repellent.

2. A process for rendering textile material water-repellent and to improve its affinity for

acid dyes which comprises impregnating textile material with a quaternary ammonium salt of a methyl halogen ether containing a basic nitrogen atom other than that of said ammonium radical, formed from a nitrile having an aliphatic radical of at least 10 carbon atoms, formaldehyde, a halogen acid, and a tertiary amine, said basic nitrogen atom being attached to said aliphatic radical, and baking the impregnated material at a temperature above about 90° C. to produce water-repellence in said textile material.

3. A process for rendering textile material water-repellent and to improve its affinity for acid dyes which comprises impregnating textile

material with a quaternary ammonium salt of a methyl halogen ether containing a basic nitrogen atom other than that of said ammonium radical, being the reaction product of octadecane nitrile, trioxymethylene, hydrochloric acid and pyridine, and baking the impregnated material at a temperature above about 90° C. to produce water-repellence in said textile material.

4. A process according to claim 1 in which cellulosic material is used and the quaternary ammonium salt contains a saturated alkyl radical of at least 10 carbon atoms in addition to at least the single basic nitrogen atom.

ERNST WALTMANN.

CERTIFICATE OF CORRECTION.

Patent No. 2,264,490.

December 2, 1941.

ERNST WALTMANN.

It is hereby certified that error appears in the printed specification of the above numbered patent requiring correction as follows: Page 1, first column, line 45, for the word "others" read --ethers--; and second column, line 40-41, for "nit ile" read --nitrile--; and that the said Letters Patent should be read with this correction therein that the same may conform to the record of the case in the Patent Office.

Signed and sealed this 6th day of January, A. D. 1942.

(Seal)

Henry Van Arsdale,  
Acting Commissioner of Patents.